

## 1

3,287,185

**PROCESS FOR IMPROVING ALLOYS BASED ON ALUMINUM, ZINC AND MAGNESIUM, AND ALLOYS OBTAINED THEREBY**

Pierre Vachet, Meudon, and Guido-Edgar Perrier, Chambéry, France, assignors to Pechiney-Compagnie de Produits Chimiques et Electrometallurgiques, Paris, France

No Drawing. Filed Nov. 14, 1963, Ser. No. 323,584  
Claims priority, application France, Nov. 15, 1962,

915,526

5 Claims. (Cl. 148—159)

The present invention concerns a process for improving alloys based on aluminum, zinc and magnesium, and the alloys obtained by applying this process.

Alloys are described by symbols prescribed by norm AFNOR number A 02-001 of May 1944; thus the symbol A-ZG describes an alloy containing aluminum, zinc and magnesium, while the symbol A-Z4G describes an alloy theoretically containing 4% of zinc and less than 4% of magnesium, the rest being made up of aluminum.

It is known that alloys of the following composition:

|           | Percent  |
|-----------|----------|
| Zinc      | 2 to 9   |
| Magnesium | 0.5 to 3 |
| Manganese | 0 to 1.5 |
| Chromium  | 0 to 0.5 |
| Titanium  | 0 to 0.5 |
| Silicon   | 0 to 1   |
| Iron      | 0 to 1   |
| Zirconium | 0 to 0.5 |
| Copper    | 0 to 3   |
| Aluminum  | to 100   |

have average mechanical and chemical properties, which make them suitable for many uses.

These alloys are based on aluminum, zinc and magnesium, the other components being optional and being essentially intended to improve the characteristics of the alloy by making the grain fine, by improving the surface of the alloy, its mechanical properties, its capacity for welding, and its suitability for anodic oxidation and surface treatment, and by increasing resistance to corrosion, with or without tension. Components other than those mentioned above may be used to obtain certain special properties.

These alloys have the common feature of being self-hardening; that is to say, they gain desirable characteristics by natural aging, after being made into a solid solution, either by an extrusion operation or separate heat treatment in a range of temperatures from about 350° to 500° C. followed by cooling in air to room temperature or by quenching or rapid cooling.

These alloys have great plasticity immediately after solution treatment, but they continue to harden slowly thereafter. The time required to obtain the final mechanical properties, which may be up to three months, often constitutes a serious disadvantage for industrial purposes.

An attempt has therefore been made to proceed with industrial tempering treatments, with the following results:

For alloys based on aluminum, zinc and magnesium without any copper and wherein the zinc content is from 2% to 4.5%, the classic example being the alloy known as "A-Z4G," no treatment of the industrial type has been found to be suitable, since such treatments only give metal mechanical properties which are far inferior to those obtained by natural aging. It is only with artificial aging processes lasting about 200 hours at a temperature of about 100° C. that desirable properties can be obtained, but such processing is commercially undesirable.

In the case of alloys of the same type, but with a zinc

## 2

content of between 4.5% and 9%, some industrially applicable artificial aging treatments may be found, but these require very exact time and temperature controls, and the time for treatment is still relatively long.

- 5 The present invention has for its object a process enabling an alloy of which the basic components are aluminum, zinc and magnesium and which has undergone quenching or cooling in air, to be given mechanical properties similar to those obtained in several months of natural aging, but in a treatment that may be carried out within a few days and preferably within 48 hours, and it is a related object to produce new and improved aluminum, zinc and magnesium base alloys and products by the described process.
- 10 In accordance with the practice of this invention, from 0.005% to 0.50% of cadmium is added to the base alloy and, after the resultant alloy has undergone a quenching or cooling in air operation, it is subjected to an artificial aging treatment at a temperature within the range of 100° to 180° C. for a time which may range from 0 up to 48 hours, and preferably 10 to 48 hours.

The alloy according to the invention is made up as follows:

|           | Percent      |
|-----------|--------------|
| Zinc      | 2 to 9       |
| Magnesium | 0.5 to 3     |
| Manganese | 0 to 1.5     |
| Chromium  | 0 to 0.5     |
| Titanium  | 0 to 0.5     |
| Silicon   | 0 to 1       |
| Iron      | 0 to 1       |
| Zirconium | 0 to 0.5     |
| Copper    | 0 to 3       |
| Cadmium   | 0.005 to 0.5 |

35 the remainder being aluminum plus small amounts of impurities.

The invention thus defined will now be explained in greater detail with the aid of the following examples, 40 which are given by way of illustration, but not by way of limitation:

An alloy of the type AZ4G and composed of the following:

|           | Percent |
|-----------|---------|
| Zinc      | 3.5     |
| Magnesium | 2.0     |
| Manganese | 0.3     |
| Chromium  | 0.15    |
| Iron      | 0.20    |
| Titanium  | 0.20    |
| Silicon   | 0.05    |
| Aluminum  | 93.60   |

will be taken as an example; it has the following properties:

55 it is solution heat treated by cooling in air after being heated to a temperature of 350° to 500° C.; it has great plasticity when freshly treated:

Breaking load .....  $R=18$  kg./sq. mm.  
Elastic limit .....  $E=9$  kg./sq. mm.  
Elongation .....  $A=22\%$

it hardens slowly after this treatment, and the following characteristics are obtained after 30 to 45 days:

65  $R=35$  kg./sq. mm.  
 $E=20$  kg./sq. mm.  
 $A=20\%$

it can easily be welded, the welded zone recovering its mechanical properties due to the self-hardening process; 70 it has good resistance to marine corrosion.

The alloy has average resistance and great ductility.

An attempt was made to obtain the characteristics obtainable by natural aging, by means of a rapid industrial treatment: the following characteristics were found after artificial aging for 200 hours at 100° C.:

$$R=36 \text{ kg./sq. mm.}$$

$$E=25 \text{ kg./sq. mm.}$$

$$A=19\%$$

The time required for such treatment is unacceptable for common commercial practice.

In the process described, the above alloy was modified by adding 0.05% of cadmium. After natural cooling, the alloy was subjected to an industrial artificial aging process lasting from about 12 to 24 hours at a temperature of 160° C. The process was effective to produce an alloy having satisfactory properties.

Table I compares the effects of these artificial aging processes, after heat treatment consisting of heating for 2 hours at 425° followed by cooling in air, firstly on a conventional A-Z4G alloy, of which the composition is given above, and secondly on the same alloy with 0.05% of cadmium added to it; the effect produced on the alloy containing cadmium by the 24-hour artificial aging process at 160° C. is virtually identical with the effect produced on the conventional alloy by the 200-hour artificial aging at 100° C.

2. The process as claimed in claim 1 in which the alloy consists essentially of:

|                                     | Percent      |
|-------------------------------------|--------------|
| Zinc-----                           | 2 to 9       |
| Magnesium-----                      | 0.5 to 3     |
| Manganese-----                      | 0 to 1.5     |
| Chromium-----                       | 0 to 0.5     |
| Titanium-----                       | 0 to 0.5     |
| Silicon-----                        | 0 to 1       |
| Iron-----                           | 0 to 1       |
| Zirconium-----                      | 0 to 0.5     |
| Copper-----                         | 0 to 3       |
| Cadmium-----                        | 0.005 to 0.5 |
| Remainder aluminum plus impurities. |              |

3. The process as claimed in claim 1 in which the alloy consists essentially of:

|                                     | Percent      |
|-------------------------------------|--------------|
| Zinc-----                           | 2.5 to 4     |
| Magnesium-----                      | 1.5 to 2.5   |
| Cadmium-----                        | 0.005 to 0.5 |
| Manganese-----                      | 0 to 0.7     |
| Chromium-----                       | 0 to 0.5     |
| Iron-----                           | 0 to 0.5     |
| Titanium-----                       | 0 to 0.5     |
| Silicon-----                        | 0 to 0.5     |
| Remainder aluminum plus impurities. |              |

TABLE I

| Alloy                         | Artificial aging 12 hours at 160° C. |                  |           | Artificial aging 24 hours at 160° C. |                  |           |
|-------------------------------|--------------------------------------|------------------|-----------|--------------------------------------|------------------|-----------|
|                               | E<br>kg./sq. mm.                     | R<br>kg./sq. mm. | Percent A | E<br>kg./sq. mm.                     | R<br>kg./sq. mm. | Percent A |
| Conventional A-Z4G            | 16.9                                 | 28.4             | 19.5      | 17.1                                 | 28.6             | 17.8      |
| A-Z4G with cadmium added----- | 25.9                                 | 34.4             | 15.3      | 27.1                                 | 35.8             | 15.5      |

The longer the time between quenching and artificial aging, the more favorable is the result.

The amount of cadmium incorporated may be from 0.005%, constituting a minimum below which no measurable effect can be ascertained, to 0.5%, the upper limit above which the alloy becomes difficult to cast. The cadmium has no perceptible undesirable effect on the welding characteristics or corrosion resistance of the alloys. The alloys can still hardened by natural aging under the same conditions as for a corresponding alloy without cadmium.

It will be understood that the invention includes the alloy and product thereof and any process in which cadmium is added to an alloy based on aluminum, zinc and magnesium with a view to permitting an artificial aging treatment of industrially acceptable duration to be carried out following a solution treatment by quenching or natural air cooling.

It will be further understood that changes may be made in the details of formulation and methods without departing from the spirit of the invention, especially as defined in the following claims.

We claim:

1. In a process of heat treating an aluminum-zinc-magnesium alloy wherein said alloy is solution heat treated followed by quenching or air cooling and artificial aging at a temperature within the range of 100-180° C. for a time within the range of 6 and 48 hours, the improvement comprising the addition of cadmium as an essential alloying element in an amount within the range of 0.005 to 0.5 percent to reduce the time required for artificially aging said alloy.

4. An alloy having the following composition:

|                                     | Percent      |
|-------------------------------------|--------------|
| Zinc-----                           | 2 to 9       |
| Magnesium-----                      | 0.5 to 3     |
| Manganese-----                      | 0 to 1.5     |
| Chromium-----                       | 0 to 0.5     |
| Titanium-----                       | 0 to 0.5     |
| Silicon-----                        | 0 to 1       |
| Iron-----                           | 0 to 1       |
| Zirconium-----                      | 0 to 0.5     |
| Copper-----                         | 0 to 3       |
| Cadmium-----                        | 0.005 to 0.5 |
| Remainder aluminum plus impurities. |              |

in which the alloy has been subjected to a solution heat treatment step which includes quenching or air cooling and which has been artificially aged to a temperature of 100° to 180° C. for a time within the range of 6 to 48 hours.

5. An alloy having the following composition:

|                                     | Percent      |
|-------------------------------------|--------------|
| Zinc-----                           | 2.5 to 4     |
| Magnesium-----                      | 1.5 to 2.5   |
| Cadmium-----                        | 0.005 to 0.5 |
| Manganese-----                      | 0 to 0.7     |
| Chromium-----                       | 0 to 0.5     |
| Iron-----                           | 0 to 0.5     |
| Titanium-----                       | 0 to 0.5     |
| Silicon-----                        | 0 to 0.5     |
| Remainder aluminum plus impurities. |              |

in which the alloy has been subjected to a solution heat treatment step which includes quenching or air cooling

and which has been artificially aged to a temperature of 100° to 180° C. for a time within the range of 6 to 48 hours.

2,915,390 12/1959 Criner 75—142  
3,031,299 4/1962 Criner 148—32.5

## FOREIGN PATENTS

## References Cited by the Examiner

5 476,930 12/1937 Great Britain.

## UNITED STATES PATENTS

1,785,774 12/1930 Hybinette 148—159 X  
2,076,577 4/1937 Kempf 75—146

DAVID L. RECK, Primary Examiner.

C. N. LOVELL, Assistant Examiner.